

E. L. WITTE.  
Method of Labeling Bottles.  
No. 204,272. Patented May 28, 1878.

*Fig: 1.*



*Fig: 2.*



WITNESSES:

*Chas. Nida*  
*C. Sedgwick*

INVENTOR:

*E. L. Witte*  
BY *M. M. M.*

ATTORNEYS.

# UNITED STATES PATENT OFFICE.

EDWARD L. WITTE, OF WHITE MILLS, PENNSYLVANIA.

## IMPROVEMENT IN METHODS OF LABELING BOTTLES.

Specification forming part of Letters Patent No. **204,272**, dated May 28, 1878; application filed February 13, 1878.

*To all whom it may concern:*

Be it known that I, EDWARD L. WITTE, of White Mills, in the county of Wayne and State of Pennsylvania, have invented a new and Improved Method of Labeling Bottles, of which the following is a specification:

Figure 1 of the drawing is a front elevation; Fig. 2, a horizontal section of the same.

The invention relates to glass labels for druggists' bottles; and it consists in a new method of labeling glass bottles by first burning the colors into the label and then melting the label into the bottle, as hereinafter described.

In the drawing, A represents a label made of glass and having its face lettered and ornamented in metallic colors fixed therein by the well-known fire-process. This label, with the

colors burned into it, is then melted into the bottle B. In this way I provide a glass bottle with a glass label in which the colors are permanently fixed, not exposed to deterioration, and practically indestructible.

Having thus described all that is necessary to a full understanding of my invention, what I claim as new, and desire to secure by Letters Patent, is—

A method of labeling glass bottles that consists in first burning the colors into the label and then melting the label into the bottle, as shown and described.

E. L. WITTE.

Witnesses:

EDWIN F. TORREY,  
C. C. JADWIN.